

## UNITED STATES PATENT OFFICE

2,019,339

## SNUFFER COMPOSITION

Frank M. Clark, Pittsfield, Mass., assignor to  
General Electric Company, a corporation of  
New York

No Drawing. Application September 29, 1934,  
Serial No. 746,274

7 Claims. (Cl. 252—1)

The present invention relates to compositions suitable for use in electrical devices, such as 5 transformers, circuit breakers, cables, and the like, for insulating and cooling purposes, and also for non-electrical purposes, for example, as lubricants.

It is the object of my invention to provide means for guarding against combustion or explosion of gaseous admixtures containing air and 10 gases given off by such compositions. My invention is of general application to materials of widely varying properties, including both hydrocarbon compounds which inherently are non-combustible in the usual sense of the word, as 15 well as ordinary combustible materials, such as mineral oil.

Various aromatic hydrocarbon compositions have been employed or proposed for industrial 20 uses which contain combined halogen in sufficiently large proportion to secure non-inflammability of the liquid mass and substantial non-inflammability and non-explosiveness of vapor derived from such compositions. However, under special conditions even such non-inflammable 25 vapors may be decomposed and yield enough finely divided carbon to result in a non-explosive, weak combustibility. For example, when such compositions are heated to a temperature depending on the volatility of the composition 30 itself and usually in the range of 110 to 200° C. and the resulting vapors come in contact with electric arcs, or sparks, then a momentary glow may occur, providing, of course, that sufficient oxygen (air) has become mixed with such vapors. Such conditions may be referred to as 35 flash-producing conditions. At higher temperatures the concentration of the halogenated vapors derived from such compositions becomes sufficiently great to diminish the air ratio to a degree sufficient to prevent "flash-producing 40 conditions" from arising.

While the combustion of carbon liberated in this way is not dangerous and cannot lead to a destructive fire, it is desirable in the operation 45 of electrical and other apparatus, that even the possibility of such weak combustion should be eliminated.

In accordance with my present invention the 50 possibility of even this sort of weak pseudo-combustibility is avoided by associating such halogenated compositions with a relatively minor proportion of a halogenated snuffer compound containing preferably at least a chemical equivalency of chlorine and hydrogen in its molecule, 55 and having a suitably chosen degree of volatility.

In carrying out my invention, the volatile snuffer compound ordinarily need be present only in relatively minor amounts, not exceeding 10% of the entire composition in order to reduce the quantity of oxygen in a body of collected 5 vapor below combustion limits. An amount of snuffer should be used which will give from about two to four per cent of vapor derived therefrom in the gas space above the level of the liquid containing the snuffer. 10

In the usual construction of electrical apparatus, such as transformers, the volume of air space does not exceed ten per cent of the volume of liquid. In such cases even a quarter per cent (0.25%) by weight of the volatile snuffer compound is capable of preventing the described 15 glow phenomenon. The amount of snuffer will depend upon circumstances in particular cases.

Halogenated olefin compounds, such as the chlorinated derivatives of the ethylenes (dichlor 20 ethylene, boiling point 37.55° C.; trichlor ethylene, boiling point 87° C.; tetrachlor ethylene, boiling point 119° C.) of the propylenes (trichlor propylene, boiling point 142° C.; tetrachlor propylene, boiling point 165° C.) and the butylenes 25 (tetrachlor butylene, boiling point 200° C.; pentachlor butylene, boiling point 185° C. under plus 60 m. m.) are illustrative of the materials which have been found to possess good snuffer action in combination with dielectric materials subject 30 to even a pseudo-combustibility.

As already indicated the essential requirement of a snuffer is that it shall possess chemical stability, that it shall be present in sufficient amount and be of such volatility that in the temperature range where pseudo-combustion of the 35 volatilized chlorinated aromatic liquid would normally be expected, the snuffer vapor will be of such concentration as to prevent flash-producing conditions. 40

The following experiment illustrates the described phenomenon: An iron tube six inches in diameter and 26 inches long is heated to a temperature within the range of 110 to 115° C. If a small amount (60 c. c.) of a liquid mixture 45 containing equal parts of trichlor benzene and pentachlor diphenyl is admitted and an electric arc is drawn in the vapor space, then a glow or pseudo-combustion effect may be observed. If the temperature of the iron tube then is increased to higher than 130 to 140° C., the vaporization of an admitted chlorinated mixture is sufficiently great to reduce the air ratio below that necessary to produce the pseudo-combustion. If now with the iron tube temperature at 55

110 to 115° C., the liquid mixture which is added contains sufficient trichlor ethylene so that at least 2% concentration of its vapors will occur in the gas space, then the pseudo-combustion 5 phenomenon is eliminated.

With pure pentachlor diphenyl, the pseudo-combustion will occur at higher temperatures. The effect of an admixed snuffer compound, however, is similar.

- 10 A snuffer compound chosen in accordance with the principles of my invention may be mixed with various halogenated compositions, for example, such compositions as are described in my prior United States Patent 1,931,373, issued 15 on October 17, 1933. Other similar compositions which may exhibit in the absence of a snuffer a momentary glow phenomenon besides trichlorbenzene and chlorinated diphenyl mixed or unmixed with one another or with other chlorinated 20 aromatic compounds, are chlorinated diphenyl methane, chlorinated diphenyl ketone, chlorinated diphenyl oxide and chlorinated naphthalene. Such compositions all are chemically inert with respect to copper and other metals present in 25 electrical devices. The addition of a halogen olefin snuffer does not depreciate this highly desirable property of chemical inertness. The halogenated olefins possess a viscosity by themselves which easily adapts these materials for dielectric 30 purposes in admixture with liquids especially in apparatus such as transformers, where low viscosity of a liquid cooling and dielectric agent is demanded for thermal reasons. Trichlor- or tetrachlor-ethylene are examples of halogenated 35 olefins suitable for dielectric use. These materials have a viscosity of about 30 seconds Saybolt Universal and show little change in viscosity over a range of temperatures. The electrical characteristics of these materials are good. Their dielectric strength, tested in a .1 inch disc electrode gap, gives a value higher than 30 kilovolts. Their dielectric constant is approximately 40 3.3 and the power factor is less than 1% at 1000 cycles, 25° C., coupled with a characteristic resistivity of about  $1 \times 10^{12}$  ohms per centimeter cube at 500 volts direct current. These characteristics make these materials particularly well adapted for admixture with other dielectric materials in transformers, circuit breakers, capacitors, cables, and the like. While particular reference has been made to snuffers containing chlorine, it should be understood that snuffer compounds containing other halogens may be 45 similarly employed.
- 50 - While my invention has been described with particular reference to the prevention of a special form of secondary combustibility of decomposed vapor derived from otherwise non-combustible halogenated cyclic hydrocarbons, the benefits of halogenated olefins as snuffers also may be obtained to a considerable degree with mate-

rials which are combustible in the ordinary sense, such for example, as mineral hydrocarbon oil. In the case of such materials "flash-producing conditions" assume the aggravated form of explosion conditions. The presence of about 5 per 5 cent of a properly chosen halogenated olefin compound (for example, trichlorethylene) in the mineral oil which commonly is used in transformers, cables, and other electric devices, will effectively reduce the explosion hazard attendant 10 upon the use of such oil.

What I claim as new and desire to secure by Letters Patent of the United States is:

1. A composition of matter comprising a hydrocarbon compound the vapor of which is combustible under flash-producing conditions and trichlorethylene within the limits of 0.25 to 10 per cent by weight associated with said hydrocarbon. 15
2. A composition of matter comprising a major proportion of halogenated hydrocarbon compound and sufficient trichlorethylene to result in the presence of about two to four per cent of the vapor thereof in a confined space above said composition. 20
3. A composition of matter consisting preponderantly or pentachlor diphenyl and trichlorbenzene and containing also less than ten per cent of a chlorinated ethylene, which has sufficiently high volatility to effectively prevent silent glow 30 combustion over said composition in a confined space. 25
4. A composition of matter comprising a carbon-containing compound the vapor of which is combustible under flash-producing conditions and less than ten per cent by weight but a substantial amount of halogenated olefin compound associated therewith, the amount and volatility of said compound being chosen to effectively prevent silent glow combustion of vapor emanating 40 from said composition. 35
5. A composition comprising a substantially non-combustible liquid hydrocarbon, the vapor of which when decomposed is capable of silent glow combustion and a minor but substantial proportion of halogenated ethylene associated with said hydrocarbon, the amount and volatility of said ethylene compound being sufficient to effectively prevent silent glow combustion. 45
6. A composition of matter comprising a major proportion of chlorinated diphenyl and a minor but substantial proportion of chlorinated olefin, which has sufficiently high volatility to prevent silent glow combustion in a space deriving vapor from said composition. 50
7. A composition of matter comprising chlorinated diphenyl and trichlor benzene and at least about a quarter per cent (0.25%) by weight of chlorinated ethylene. 55

FRANK M. CLARK. 60

CERTIFICATE OF CORRECTION.

Patent No. 2,019,339.

October 29, 1935.

FRANK M. CLARK.

It is hereby certified that error appears in the printed specification of the above numbered patent requiring correction as follows: Page 2, second column, line 27, claim 3, for "or" read of; and line 44, claim 5, for "cable" read capable; and that the said Letters Patent should be read with these corrections therein that the same may conform to the record of the case in the Patent Office.

Signed and sealed this 10th day of December, A. D. 1935.

(Seal)

Leslie Frazer  
Acting Commissioner of Patents.